

## UNITED STATES PATENT OFFICE

2,488,515

## UTILIZATION OF WASTE WAX PAPER

Laurence R. Sherman, Glens Falls, N. Y., and W. Ronald Benson, Seattle, Wash., assignors of one-half to Nopco Chemical Company, a corporation of New Jersey and one-half to Crown Zellerbach Corporation, San Francisco, Calif., a corporation of Nevada

No Drawing. Application May 10, 1945,  
Serial No. 593,104

6 Claims. (Cl. 92—1.6)

1

The present invention relates to the reclaiming and utilization of waste wax paper. More particularly the present invention relates to the utilization of wax cuttings and the like known in the art as wax broke for the manufacture of any other type of paper either alone or in admixture with additional wood fiber or other forms of paper.

Utilization of waste wax paper, wax trimmings and the like has been a considerable problem in the art inasmuch as the wax on this paper would be set free during subsequent processing on the screens and other parts of paper making machines, and the finished paper, even though the wax broke had been admixed with other pulp, would show evidences of wax spots and other deformities in the paper surface.

Various processes have been suggested for utilizing waste wax broke; for example, in U. S. Patent No. 2,183,259 there is disclosed a process for recovering wax broke which consists of mechanically disintegrating the wax broke in water and gradually raising the temperature of the water to a point above the melting point of the wax. Thereafter an emulsifier is added which consists primarily of a mixture of sulfonated oils, such as sulfonated olive oil, cottonseed oil, sperm oil, etc. with mahogany soaps. Although this process has been found commercially acceptable for reclaiming and reusing wax broke, the resultant fibers have not been generally capable of use in any except the heavier forms of paper manufacture. Furthermore, during warm weather at times wax deposits on the screens and other portions of the paper making apparatus would cause trouble.

In accordance with the present process, however, it has been discovered that this action may be prevented if the wax broke is treated after heating with a suitable proportion of a cationic surface active agent of the character to be hereinafter described. The action of the cationic matter appears to be entirely dissimilar to that of the emulsifying agents disclosed in the aforementioned patent in that no true emulsion of the wax is formed and the wax cannot be washed from the paper fibers. Instead the wax and cationic surface active substance appear to be fixed on the paper fibers and homogeneously retained thereon. However, the resultant treated fibers do not give up their wax so that there is no troublesome deposit of wax on the paper making machines nor are there any wax spots apparent in the finished paper. The resultant paper fibers with the wax fixed thereon can be used

either by themselves to form sheets or, in the event such a high proportion of wax size is not desired, the fibers may be combined with other paper fibers or other forms of fiber in any suitable proportion.

It is one of the objects of the invention, therefore, to provide a novel process for the utilization of wax paper waste, i. e. wax broke.

A second object of the present invention is to provide a novel process which includes fixing the wax derived from wax broke directly on the fibers in such a manner that no wax deposits are formed in the paper making machinery or wax spots in the finished sheet.

Other objects and advantages of the present invention will become apparent from the present description and claims.

In practicing the present process a suitable quantity of wax broke is charged into a beater or other paper making apparatus capable of disintegrating the same. Thereafter the beater is heated to a temperature sufficient to melt the wax. Inasmuch as the type of wax used in making waste paper generally has a melting point of approximately 120° F., the beater is brought to a temperature above this point, such as approximately 130–160° F., by the use of steam or by other heating means. Thereafter a cationic surface active material of the type hereinafter to be described is added to the proportion of at least 3% by weight of the wax. The cationic substance apparently fixes the residual wax on the fibers and permits the use of the so-treated broke in paper manufacture in the usual manner.

The cationic surface active agents used in accordance with the present invention include certain amino-amides, glyoxalidines cyclized from those amino-amides, and the solubilized derivatives of either. The amino-amides may best be described by the general formula:



wherein R<sup>1</sup> represents an aliphatic chain containing from 7 to 23 carbon atoms; R<sup>2</sup> denotes a substituent selected from the group consisting of hydrogen and alkylol groups containing 1 to 3 carbons, and n is a number selected from the group consisting of 2 and 3 when R<sup>2</sup> stands for hydrogen and n is a number selected from the group consisting of 1, 2 and 3 when R<sup>2</sup> represents an alkylol radical. Glyoxalidines may be formed from amino-amides of the above formula by internal condensation wherein the carboxyl carbon

atom of the amido group is linked to the nitrogen atom of the nearest amino group in the molecule. This glyoxalidine ring formation occurs when the oxygen and hydrogen atoms of the amido group combine with a hydrogen atom of the nearest amino group thereby liberating a molecule of water. Further, compounds corresponding to soluble acid salts or alkylated derivatives of the above type of compound may be used. These may be produced by treating a compound of the general formula above described with an aliphatic monocarboxylic acid of from 1 to 3 carbon atoms such as acetic, formic, glycolic, etc. or with a suitable ester of a mineral acid, as, for example, diethyl sulfate, triethyl phosphate, ethyl iodide, etc. The resultant solubilized compounds may then be illustrated by the general formula:



where  $\text{R}^1$ ,  $\text{R}^2$  and  $n$  have the values assigned previously,  $\text{R}^3$  denotes a substituent selected from the group consisting respectively of hydrogen, when  $\text{R}^3\text{Z}$  is a 1 to 3 carbon aliphatic monocarboxylic acid, and an aliphatic alkyl group of from 1 to 3 carbon atoms, when  $\text{R}^3\text{Z}$  is an ester of a mineral acid with a 1 to 3 carbon aliphatic alcohol, and  $\text{Z}$  is selected from the group consisting of the respective residues of said acid and said ester; and where the formula also encompasses the same derivatives of glyoxalidines produced from the amino-amides prior to addition of the  $\text{R}^3$  and  $\text{Z}$  radicals by linking the carboxyl carbon atom with the nitrogen atom of the nearest amino group accompanied by liberation of a molecular proportion of water.

In preparing the cationic compound which fixes the residual wax on the fibers in accordance with the present invention, a suitable fat or fatty acid is reacted with a polyalkylene polyamine compound in order to form an amino-amide, or in the alternative, the fatty acid or fat is reacted with an alkylene alkylol polyamine or a polyalkylene alkylol polyamine compound. Thereafter, the amino-amide may be heated to a relatively high temperature to drive off water in order to form a cyclic compound. The amino-amide, or the cyclic glyoxalidine compound equivalent to the amino-amide, may then be treated with an agent rendering the compound water soluble, such as a suitable ester of a mineral acid, for example, diethyl sulphate, triethyl phosphate, ethyl iodide, or an aliphatic monocarboxylic acid of from 1 to 3 carbon atoms such as acetic, formic, glycolic, etc. or the amide or glyoxalidine may be added first to the paper fibers and wax and thereafter the acid.

In general, temperatures in the neighborhood of 200° C. or from 150 to 210° C. are utilized for the amidification, and in the event the cyclic compound is desired, temperatures in the neighborhood of 300° C. are used. Various polyalkylene polyamine, alkylene alkylol polyamine or polyalkylene alkylol polyamine compounds having from 2 to 4 amino groups may be used as, for example, diethylene triamine, ethanol ethylene diamine, ethanol diethylene triamine, triethylene tetramine, etc. Almost any fatty acid or fatty acid glyceride having from 8 to 24 carbon atoms in the chain may be utilized as the fatty acid portion of the compound. Thus, oleic acid, ricinoleic acid, lauric acid, stearic acid, palmitic acid, etc. are examples of the fatty acids which may

be utilized in preparing the amino-amide compound.

The following specific examples, wherein all proportions are expressed in terms of weight, serve to illustrate but are not intended to limit the present invention.

#### Example I

74.8 parts by weight of hydrogenated soybean oil and 25.2 parts of ethanol ethylene diamine were condensed in a closed vessel at 150° C. for from 6 to 8 hours. The product was believed to consist largely of an amino-amide having the following formula:



Thereafter 17.4 parts of the above amino-amide were placed in a stainless steel vessel and melted. A mixture of 3.7 parts of 70% acetic acid and 78.9 parts of water preliminarily heated to 85° C. were then added to the melt and the entire mass stirred until a homogeneous gel formed. This gel was believed to contain substantial amounts of a compound having the formula:



500 grams of waste wax cuttings containing approximately 12% wax were slowly charged into a Valley 1 1/2 pound Niagara beater containing 2300 grams of water at 100° F. Three grams of the cationic agent produced as above set forth were then added and the heating continued with a one pound weight on the lever arm of the beater while heating with steam to a temperature of 140° F. The time of heating and beating was approximately 30 minutes. No scum formed on the surface and no wax break appeared when a small amount of the suspension was poured into cold water. Thereafter hand sheets were made from the suspension of fibers and wax. These sheets had a good appearance and were entirely free from wax spots and the like.

#### Example II

78.3 parts by weight of peanut oil and 27.5 parts by weight of diethylene triamine were heated together to a temperature of about 150° C. in a closed vessel and held at this temperature for about 6 to 8 hours. Thereafter the amino-amide was added to wax broke in a beater as set forth in Example I. The only difference in the procedure being that after the amino-amide was added to the wax broke and water at 140° F. and beating continued for about 30 minutes, sufficient acetic acid to bring the pH of the slurry from pH 8 to pH 6 was added and the slurry was again beaten for about 30 minutes. Sheets made from this slurry were also entirely satisfactory and no wax deposits in the beater were observed.

#### Example III

78.3 parts by weight of peanut oil and 27.5 parts by weight of diethylene triamine were heated together to a temperature of between 180 and 190° C. and held at this temperature for 20 minutes. Thereafter the reaction mixture was rapidly heated to 300° C. and the evolved water was

collected in a moisture trap. When 5.8 parts of aqueous condensate were collected, the heat was shut off and the product allowed to cool. The resultant product was believed to have the following formula:



where R represents the alkyl radicals of peanut oil.

500 grams of waste cuttings were treated with the above cationic agent in a manner similar to that of Example I. The resulting hand-made sheets were entirely satisfactory and free from wax spots.

Having described our invention, what we claim as new and desire to secure by Letters Patent is:

1. A process for reclaiming wax paper broke, the steps consisting of forming a suspension in water of the fibers of the wax paper broke by disintegrating the broke in water heated to a temperature sufficiently high to melt the wax, and fixing the wax on the fibers by adding a cationic surface active substance to the fiber and wax suspension, said cationic substance being selected from the group consisting of amino-amides having the general formula:



and salts of said amino-amides having the general formula:



where R<sup>1</sup> represents an aliphatic chain containing from 7 to 23 carbon atoms, R<sup>2</sup> denotes a substituent selected from the group consisting of hydrogen and alkylol groups containing 1 to 3 carbon atoms, and n is a number selected from the group consisting of 2 and 3 when R<sup>2</sup> stands for hydrogen and n is a number selected from the group consisting of 1, 2 and 3 when R<sup>2</sup> represents an alkylol radical, R<sup>3</sup> denotes a substituent selected from the group consisting respectively of hydrogen, when R<sup>3</sup>Z is a 1 to 3 carbon aliphatic monocarboxylic acid, and an aliphatic alkyl group of from 1 to 3 carbon atoms, when R<sup>3</sup>Z is an ester of a mineral acid with a 1 to 3 carbon aliphatic alcohol, and Z is selected from the group consisting of the respective residues of said acid and said ester.

2. A process according to claim 1 in which the quantity of said cationic surface active substance added is at least 3% of the weight of the wax present in the suspension.

3. A process for reclaiming wax paper broke, the steps consisting of forming a suspension in water of the fibers of the wax broke by disintegrating the broke in water heated to a temperature sufficiently high to melt the wax, and fixing the wax on the fibers by adding a cationic surface active substance to the fiber and wax suspension and thereafter adding an aliphatic monocarboxylic acid containing from 1 to 3 carbon atoms per molecule to the suspension to reduce the pH value to approximately 6, said cationic substance be-

ing selected from the group consisting of amino-amides having the general formula:



where R<sup>1</sup> represents an aliphatic chain containing from 7 to 23 carbon atoms, R<sup>2</sup> denotes a substituent selected from the group consisting of hydrogen and alkylol groups containing 1 to 3 carbon atoms, and n is a number selected from the group consisting of 2 and 3 when R<sup>2</sup> stands for hydrogen and n is a number selected from the group consisting of 1, 2 and 3 when R<sup>2</sup> represents an alkylol radical.

4. A process for reclaiming wax paper broke, the steps consisting of forming a suspension in water of the fibers of the wax paper broke by disintegrating the broke in water heated to a temperature sufficiently high to melt the wax, and fixing the wax on the fibers by adding the acetic acid solubilized derivative of ethanol amino ethylene stearamide to the suspension.

5. A process for reclaiming wax paper broke, the steps consisting of forming a suspension in water of the fibers of the wax paper broke by disintegrating the broke in water heated to a temperature sufficiently high to melt the wax, and fixing the wax on the fibers by adding ethanol amino ethylene stearamide to the suspension and thereafter adding acetic acid to the suspension.

6. A process according to claim 5 in which the quantity of ethanol amino ethylene stearamide added is at least 3% of the weight of the wax present in the suspension.

LAURENCE R. SHERMAN.  
W. RONALD BENSON.

#### REFERENCES CITED

40 The following references are of record in the file of this patent:

#### UNITED STATES PATENTS

| Number       | Name         | Date          |
|--------------|--------------|---------------|
| 4,970,426    | Levin        | Aug. 14, 1934 |
| 1,992,589    | Tucker       | Feb. 26, 1935 |
| 2,096,129    | Neitzke      | Oct. 19, 1937 |
| 2,183,259    | Hill         | Dec. 12, 1939 |
| 2,186,609    | Kress        | Jan. 9, 1940  |
| 2,206,090    | Haggenmacher | July 2, 1940  |
| 2,268,273    | Wilkes       | Dec. 30, 1941 |
| 2,277,788    | Shipp        | Mar. 31, 1942 |
| 2,343,090    | Smith        | Feb. 29, 1944 |
| 2,343,095    | Smith        | Feb. 29, 1944 |
| 55 2,347,178 | Fritz et al. | Apr. 25, 1944 |
| 2,401,027    | Tausch       | May 28, 1946  |
| 2,442,972    | Edelstein    | June 8, 1948  |

#### FOREIGN PATENTS

| Number  | Country       | Date          |
|---------|---------------|---------------|
| 319,745 | Great Britain | Dec. 29, 1930 |

#### OTHER REFERENCES

- Technical Association Papers, Series 22, pp. 264-267 (1939).  
 Paper Trade Journal, Aug. 22, 1940, pp. 30, 31.  
 Rayon Textile Monthly, Mar. 1944, p. 79.  
 Journal of Society Chemical Industries, Apr. 1938, p. 117.  
 70 Paper Trade Journal, June 29, 1944, pp. 27-32.  
 Industrial and Engineering Chemistry, Jan. 1941, pp. 16-22.